

Feb. 28, 1933.

A. C. FISCHER

1,899,435

EXPANSION JOINT

Original Filed May 5, 1926

Fig. 1.



Fig. 2.



Inventor:  
Albert C. Fischer,

By *Albert C. Fischer*  
Atty.

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## EXPANSION JOINT

Application filed May 5, 1928, Serial No. 106,985. Renewed June 30, 1930.

The present invention relates to expansion joint and the like composition material, and has particular reference to the use of matted fibrous material in thin foliations, preferably 5 in 2 and 3 inch lengths as a filling medium for such material. As described in the present invention vegetable fibrous matter when being prepared for insulation material is degummed by treating with caustic and water, 10 is then matted by driving thru rolls after being washed and placed in heating ovens for drying. This process distinguishes somewhat over the felting process in which fibres in their finally or ultimately divided state are 15 felted together after proceeding thru beaters, and are then interlaced and gathered together in a continuous felt sheet.

This invention consists in taking foliations of matted fibrous material of preferably long, 20 linear dimension, waterproofing same with an excess waterproofing and matting same together under pressure, the waterproofing material adhering the foliations together, making a dense waterproofed binding medium intermediate of the irregularly matted foliated sections of the matted fibrous material. These waterproofed mats may be internally waterproofed or not as desired. This built-up highly resilient foliated structure of 30 ductile binding material and resilient foliated fibrous material provides a most excellent expansion joint.

## In the drawing:

Fig. 1 is a perspective view of strip embodying the present invention; and

Fig. 2 is a plan view of one of the foliated pieces which is incorporated in the binder.

Suitable means are provided for waterproofing the fibrous material internally by 40 using an oil or a low melting point saturant, such for instance as is used in saturating roofing felt, which is usually of a much lower melting point than the coating which is placed on the outside of roofing paper. This, 45 of course, makes the mat flexible and more readily enters the pores of the fibrous mat. If it is desirable these fibrous mats may be taken in an unsaturated state and coated with a high melting point bituminous material, or 50 alternatively, by using a high melting point

bituminous material the fibrous material can be readily water-proofed by a dense coating of a high melting point material. Also in these fibrous mats, a process may be followed in which the fibrous mats are treated with 55 lighter oils, as described, and then later coated with a high melting point bituminous waterproofing material, said mats thus being formed into a matted sheet by pressure rolls.

A suitable source for the material for forming the mats consists of the trimmings available from manufacturing plants preparing this material, by which method pieces of the matted fibre up to 2 and 3 inches long can readily be secured in volume. 60

My improved expansion joint thus consists of fibrous material, preferably vegetable fibrous material, formed into relatively small mats, which mats are individually coated with compressible bituminous material, 70 preferably of high melting point, and all of these mats are then firmly adhered together into desired form by a binder, preferably bituminous material, thus forming foliations preferably of long linear dimension and separated by zones of compressible bituminous material. It will be appreciated that such a construction for an expansion joint provides a light and strikingly resilient body which provides the maximum compressibility and 80 expansibility so necessary to the demands of an expansion joint. By providing the separate mats with coatings, particularly of high melting point asphalt, the separate mats are firmly bound together, and full effect is given 85 to each cushioning function of the separate mats thru the intermediary of the intervening coatings of bituminous material.

## I claim:

1. A foliated structure consisting of matted vegetable fibrous material, alternating in foliations of long linear dimension with a ductile waterproofed material, said fibrous foliations lying in overlapping irregular position intermediately of layers of waterproofing material, and formed into strips of expansion joint. 90

2. A preformed expansion joint consisting of a structure of foliations of long linear dimension, said foliations consisting of 100

fibrous matted material, lying in irregular overlapping position intermediately layers of waterproofing ductile material, said foliations of fibrous material being entirely surrounded by the ductile material.

3. An expansion strip formed by combining numerous foliations of long linear dimension consisting of fibrous matted material individually coated with bituminous material, pressed into strips lying in irregular overlapping position and held together by a suitable binder adapted for use as expansion joints.

4. An expansion strip formed by combining numerous waterproofed foliations of fibrous matted material, said foliations being of long linear dimension, as described, coated and adhered together in irregular overlapping position by a suitable binder, for use as expansion joints.

5. A preformed expansion joint comprising individual mats of fibrous material coated with high melting point asphalt and united so that the separate foliations lie in irregularly overlapping relation with the bituminous material separating the individual foliations.

6. In a preformed expansion joint strip a fibrous body waterproofed with a high melting point bituminous material, said waterproofed body being further waterproofed with a waterproofing coating of ductile character.

7. In a preformed expansion joint strip a fibrous body coated with a high melting point bituminous material, said bituminous coated fibrous material being further waterproofed with a layer of ductile character.

Signed at Chicago, Illinois this 20 day of April, 1926.

ALBERT C. FISCHER.

45

50

55

60

65